

## UNITED STATES PATENT OFFICE.

RALPH AUSTIN LONG, OF TAMAQUA, PENNSYLVANIA, ASSIGNOR TO ATLAS POWDER COMPANY, OF WILMINGTON, DELAWARE, A CORPORATION OF DELAWARE.

## COMMERCIAL BLASTING EXPLOSIVE.

No Drawing.

Application filed May 13, 1925. Serial No. 30,087.

This invention relates more particularly to commercial blasting explosives of varying strengths, containing from about 11% to about 47% ammonium nitrate. 5 Ammonium nitrate has been used for years as a substitute for nitroglycerine in commercial dynamite. It has the advantage of being cheaper than nitroglycerine and producing explosives safer to handle and less 10 easily ignited. One drawback to ammonium nitrate is that it contributes very little to the propagation sensitiveness of explosives and therefore must be used in conjunction with a sensitizer consisting usually of an explosive organic nitrate or nitrates or some explosive nitro aromatic compound or compounds or both. 15

Under normal conditions these sensitizing explosives are much more costly, strength for strength, than ammonium nitrate. Also nitroglycerine or a mixture of nitroglycerine with nitrated polymerized glycerine, which are the most common explosive organic nitrates used 20 as sensitizers, have the disadvantage of causing severe headaches to those handling them, are extremely sensitive to shock, and become quite dangerous to handle when frozen. These undesirable properties are inherent 25 in the explosives containing them to an extent depending, in a general way, on the quantity used, although not necessarily in direct proportion to that quantity. In explosives containing, for example, 60%, 50% or 40% nitroglycerine or some similar explosive organic nitrate, it would be a difficult 30 matter to determine much difference between them in regard to such properties. But as the nitroglycerine content is further reduced these undesirable properties become less noticeable, and especially so during successive 35 reductions below about 12%. There is a limit however, below which any further reduction in the nitroglycerine content seriously interferes with the propagation sensitiveness. 40

By extensive thought and a vast number of tests on various combinations of the explosive ingredients, I have succeeded in obtaining satisfactory propagation sensitiveness 45 although reducing the quantity of sensitizing compound or compounds to a greater extent than has heretofore been consid-

ered practicable in explosives containing from about 11% to about 47% ammonium nitrate. I have therefore obtained greater 55 economy in manufacture and in the use of ingredients, while at the same time, I have produced an explosive that is less sensitive to shock, less easy of ignition, one which has much less tendency to freeze, (is in fact, 60 practically non-freezing), and one which has much less tendency to cause headaches in handling.

The strength of my explosive is varied 65 essentially by varying the ammonium nitrate content, while explosive organic nitrates are used in an amount sufficient to give considerable propagation sensitiveness, but not in an amount sufficient to interfere with the other desirable features of my explosive such as its great economy, safety, and reduced tendency to cause headaches. Explosive nitroaromatic compounds may be used in a limited amount as an additional sensitizer and to lower the freezing point. Inorganic nitrates may also be used as a filler 75 and to provide the desired amount of oxygen, together with various well known ingredients of a non-explosive but combustible nature such as ground wood, sulphur, etc. 80

Briefly, my explosive contains a sensitizer which is never in excess of 12 per cent and which consists of from four and one-half to eight and one-half per cent, (4½% to 8½%) of an explosive liquid organic nitrate or a mixture of explosive liquid organic nitrates and from zero to seven and one-half per cent, (0 to 7½%) of an explosive nitroaromatic compound or compounds such as trinitrotoluene for example, 90 together with from about eleven to about forty-seven per cent, (11% to 47%) ammonium nitrate, depending on the strength desired, together with a non-explosive inorganic nitrate or nitrates to act as a filler 95 and supply a desired amount of oxygen. In addition to these, various quantities of non-explosive combustible materials may be added for the purpose of manipulating the density or oxygen balance without departing from the spirit of my invention. Where the term nitrate is used in the accompanying claims, it is to be understood to include mixtures of nitrates. 100

The following are typical formulae of my explosives:

|                                                       |    | Per cent. |      |
|-------------------------------------------------------|----|-----------|------|
| Ammonium nitrate                                      | 47 | 40.5      | 31   |
| 5 Mixture of nitroglycerine and tetranitrodiglycerine | 8  | 8         | 8    |
| Sodium nitrate                                        | 33 | 39        | 47.5 |
| Nitroaromatic compound                                | 2  | 2         | 2    |
| 10 Non-explosive combustibles (ground wood, etc.)     | 10 | 10.5      | 11.5 |

Although I have used, in these examples, a mixture of nitroglycerine and tetranitrodiglycerine as the liquid explosive organic nitrate, I may also use nitroglycerine (glycerine trinitrate) alone, or mixtures of glycerine trinitrate with other liquid explosive organic nitrates, such as the glycol dinitrates, chlorhydrindinitrate, and suitable 15 nitrated carbohydrates, or I may use explosive liquid organic nitrates exclusive of glycerine trinitrate. 20

Having described my invention, what I claim is:

1. A blasting explosive of the character 25 described, comprising nitro-glycerine up to 8%, ammonium nitrate, trinitrotoluene and a non-explosive combustible, the nitroglycerine and the trinitrotoluene complementally constituting a sensitizer not in excess of 12 30 per cent of the whole, and in which the nitroglycerine is in excess of the trinitrotoluene.

2. A blasting explosive of the character 35 described, comprising the following ingredients combined in substantially the proportions stated, viz: ammonium nitrate up to 47 per cent; nitroglycerine not to exceed 8 per cent; sodium nitrate from 33 to 47.5 per cent; trinitrotoluene 2 per cent, and, a non- 40 explosive combustible.

In testimony whereof he affixes his signature.

RALPH AUSTIN LONG.